# EUROPEAN PATENT SPECIFICATION

(11) **EP 3 995 625 B1**
(45) Date of publication and mention of the grant of the patent: **03.04.2024**
(21) Application number: 21201022.7
(22) Date of filing: 05.10.2021
(51) Int. Cl.: D06M 13/395, D06M 15/564, D06M 15/227

(54) **METHOD FOR WATERPROOFING FABRIC GARMENTS**
VERFAHREN ZUM HYDROPHOBIEREN VON KLEIDUNGSSTÜCKEN
PROCÉDÉ D'IMPERMÉABILISATION DE VÊTEMENTS EN TISSU

(30) Priority: 04.11.2020 IT 202000026272
(43) Date of publication of application: 11.05.2022
(73) Proprietor: Ratti S.p.A. Società Benefit, 22070 Guanzate (CO) (IT)
(72) Inventor: GIDARO, Pino, I-22070 Guanzate, COMO (IT); VALSECCHI, Arianna, I-22070 Guanzate, COMO (IT); GEROSA, Marco, I-22070 Guanzate, COMO (IT)
(74) Representative: Long, Giorgio

(56) References cited:
- WO-A1-2016/061099
- US-B1- 6 238 745

## Description

The present invention relates to a method for waterproofing fabric products, in particular garments, in particular for restoring the water-repellent functionality of used garments.

Waterproofed garments are widely known and used. However, the water-repellent functionality degrades due to the number of washes to which the garment is subjected, exposure to atmospheric agents and use.

Products are available on the market which, applied to the used garment in a spraying mode or in a domestic washing machine, restore the water-repellent functionality.

However, the known household methods give a water-repellency of poor duration over time, expose the user in the domestic environment to potentially harmful effluents, and if carried out in a washing machine, include an excessive consumption of water.

In this context, it is the technical task underlying the present invention to provide a method which can be performed in an industrial environment and allows to overcome the drawbacks of the known art providing a restoration of the water-repellency of a garment for a sufficiently long period of time, at a low cost and environmental impact.

The specified technical task is substantially achieved by a method comprising the technical features set out in one or more of the appended claims, the definitions of which form an integral part of the present description.

WO 2016/061099 A1 discloses a method for giving water-repellant properties to textile products comprising the steps of the preamble of claim 1.

Therefore, the present invention relates to a method for giving water-repellent properties to textile products according to the invention and comprises the following operating steps:
A) providing new or used textile products;
B) washing said textile products;
C) drying said washed textile products;
D) waterproofing said dried textile products;
E) drying said waterproofed textile products;
F) heat-treating the waterproofed and dried textile products, characterized in that the waterproofing step D) is carried out, preferably by spraying, using a waterproofing composition comprising or consisting of:
   i) a suspension or nanosuspension of silicon dioxide;
   ii) hydrocarbon dendrimers or aminated hydrocarbon dendrimers in a hydrocarbon matrix;
   iii) polyfunctional isocyanate polymer containing hexamethylene diisocyanate.

Further features and advantages of the present invention will become more apparent from the indicative and thus non-limiting description of a preferred, but not exclusive embodiment of the invention, with reference to the drawings, in which:
figure 1 depicts a diagrammatic view of a plant for carrying out the method according to the invention
The method for giving water-repellent properties to textile products according to the invention comprises the following operating steps:
A) providing new or used textile products;
B) washing said textile products;
C) drying said washed textile products;
D) waterproofing said dried textile products;
E) drying said waterproofed textile products;
F) heat-treating the waterproofed and dried textile products.

The term "textile products" according to the present invention means in particular items of clothing, such as raincoats, coats, down jackets, anoraks, capes, hats, caps, shawls, duster coats, jackets, pants, padded or unpadded vests, etc. The term "textile products" further includes blankets, sleeping bags, tents, curtains, and any other used fabric products which require a waterproofing treatment.

The term "giving water-repellent properties" according to the present invention means both a first waterproofing on a new or used product which has not been previously waterproofed, and a restoration of the waterproofing properties which may have faded following prolonged use or washing.

Figure 1 diagrammatically shows a plant 1 for carrying out the method of the invention.

Step B) of washing is especially important in the case of used items as, in order to obtain a good water-repellent effect on a fabric, it is essential to eliminate the substances from the fabric which could interfere with the waterproofing treatment.

In particular, the interfering substances resulting from daily use can be:
- residues of surfactants, in particular highly wetting anionic surfactants, deriving from washing with poor rinsing;
- residues of deodorant;
- residues of insect-repellent substances;
- various kinds of dirt.

With reference to figure 1, the washing step B) can be carried out in an oval machine 2, for example an AOM-C WOOL machine from FLAINOX. Such an apparatus operates discontinuously and consists of an oval stainless steel container into which the textile products to be treated are manually loaded.

The movement of the bath is imparted by four stainless steel blades which rotate inside the oval container, on a horizontal shaft driven by an electric motor, with the aim of circulating the bath and the textile products to be treated in the same direction.

The bath temperature can be increased by indirect heating, obtained with heat exchange through the passage of steam inside a coil placed on the bottom of the oval container.

The bath temperature can also be decreased by passing cold water inside the heat exchanger.

The washing step B) preferably comprises the following steps:
b1) washing the textile products with low-surfactant detergent
b2) first rinsing
b3) washing with surfactant extraction agent
b4) second rinsing
b5) optionally, third rinsing.

Step b1) is preferably carried out with an aqueous mixture of fatty acid starches and dispersants. An example is the commercial product Tanaterge EF from the company New Tanatex S.p.A. Such a detergent features excellent emulsifying power towards oils and paraffins, excellent suspending power for the removed impurities, a good soaping effect, good biodegradability, is low foaming and has low wetting power.

The concentration of detergent in water is preferably between 1 g and 3 g per liter of water.

Step b3) is preferably carried out with a condensation product of aromatic sulfonic acids and formaldehyde comprising sodium naphthalene sulfonate. An example of such a compound is the commercial product Erional RF from the company Huntsman, which comprises synthetic tannin and has a strong dispersing power so as to solubilize and extract the surfactants blocked inside the fibers.

The concentration of extracting agent in water is preferably between 1 g and 3 g of extracting agent per L of water.

In step b3), it is important that the pH of the bath is about 5. For example, 80% acetic acid can be used as an acidifying agent.

Steps b2), b4) and b5) of rinsing are carried out with water. The third rinsing step b5) is optional and will be carried out for example if the weight of the textile products being processed is high.

According to a particular embodiment of the invention, step B) includes:
i) weighing the dry textile products
ii) filling the machine with an amount of softened water at a ratio of 40:1 on the weight of the dry textile product
iii) adding a 2 g amount of detergent, preferably Tanaterge EF, for each L of bath
iv) actuating the bath movement blade, so as to circulate and homogenize the washing bath
v) adding the textile products, preferably one at a time so that they are evenly distributed in the tank
vi) heating the bath up to a temperature of 30-40°C, for example based on the maintenance tag of the textile products
vii) once the treatment temperature has been reached, allowing the bath and textile products to circulate for about 20 minutes
viii) after this time, draining the bath, leaving the textile products therein
ix) rinsing the washed textile products by filling the machine with untreated water at a ratio of 40:1 on the weight of the dry textile products, at room temperature and for a residence time of about 10 minutes
x) removing the textile products from the tank
xi) draining the bath
xii) filling the machine with an amount of softened water at a ratio of 40:1 on the weight of the dry textile products
xiii) adding a 2 g amount of surfactant extraction agent, preferably Erional RF, pre-diluted 1:1 with cold softened water, for each L of bath
xiv) controlling the pH value of the bath, for example using a litmus paper
xv) if needed, adjusting the bath to the pH value ~ 5 by adding an appropriate amount of 80% acetic acid
xvi) inserting the wet textile products removed in step 10 into the tank
xvii) increasing the temperature to no more than 40°C
xviii) allowing the textile products to turn in the bath at this temperature for about 30 minutes
xix) draining the bath
xx) filling the machine with an amount of untreated water at a ratio of 40:1 on the weight of the dry textile products
xxi) cold-treating the textile products for about 10 minutes
xxii) based on the type of textile products being processed, considering whether to repeat another rinse
xxiii) removing the textile products from the tank and placing them on special carriages.

It should be noted that the washing step B) can also be carried out in a site other than that in which the remaining steps of the method are carried out. For example, the washing step B) can be carried out in specialized laundries, for example industrial laundries.

Step C) of drying preferably comprises the following steps:
c1) spinning the textile products washed according to step B)
c2) drying the spun textile products.

With reference to figure 1, step c1) can be carried out in a centrifuge 3 for fabrics, for example an ESH.CC hydroextractor from the company Pozzi Leopoldo s.r.l. The hydroextractor is a machine for discontinuous processing, consisting of a stainless steel body provided with an openable upper lid, inside which a perforated basket is inserted which rotates on a vertical axis driven by an electric motor.

The spinning speed in step c1) is no higher than 500 rpm.

With reference to figure 1, step c2) can be carried out in a dryer 4 for fabrics, for example a dryer D 110 from the company Renzacci S.p.A. The dryer (or tumbler) is a machine for discontinuous processing, consisting of a closed and heated metal body, in which a perforated metal basket is inserted which rotates on a horizontal axis driven by an electric motor. The internal heating of the machine is obtained by a heat exchanger, inside which steam circulates.

The drying temperature in step c2) is preferably not more than 40°C.

Step D) of waterproofing is carried out using a waterproofing composition comprising or consisting of:
i) a suspension or nanosuspension of silicon dioxide;
ii) hydrocarbon dendrimers or aminated hydrocarbon dendrimers in a hydrocarbon matrix;
iii) polyfunctional isocyanate polymer containing hexamethylene diisocyanate.

The waterproofing composition preferably comprises or consists of:
- 75-85% by weight of silicon dioxide suspension or nanosuspension
- 14-23% by weight of hydrocarbon dendrimers or aminated hydrocarbon dendrimers in a hydrocarbon matrix
- 0.5-3% by weight of polyfunctional isocyanate polymer solution containing hexamethylene diisocyanate.

In a preferred embodiment, the waterproofing composition consists of:
- 79% by weight of the product Nanopool^{®} Fibre Protect
- 20% by weight of the product Ruco-Dry^{®} DHY
- 1% by weight of the product Arkophob^{®} XLR.

The product Nanopool^{®} Fibre Protect is marketed by APC Italia s.r.l. Silicon oxide simultaneously gives the fabric hydrophobicity and oleophobicity, is safe for both humans and the environment and can be used on practically all fabrics with natural fibers, but when used alone, it shows poor resistance to maintaining the performance thereof on synthetic fibers, especially polyamides.

The waterproofing composition of the present invention solves such a technical problem by virtue of the components ii) and iii) described above, which give rise to a low temperature cross-linking, compatible with the treatment of the used textile products according to the invention.

The product Ruco-Dry^{®} DHY is marketed by the company Rudolf Group.

The product Arkophob^{®} XLR is marketed by the company Archroma.

The amount of waterproofing composition used in step C) is preferably 70-90% by weight, more preferably about 80% by weight, with respect to the weight of the dry textile products.

The application of the waterproofing composition is preferably carried out by spraying and can be done with the following methods:
- manually by an operator with a spray gun in a vacuum cabin
- automated with anthropomorphic robot provided with a spray applicator in a vacuum cabin
- automated with closed machine provided with a spray applicator.

Preferably, with reference to figure 1, the application of the waterproofing composition on the washed and dried textile products is carried out by means of a spraying machine 5 for discontinuous processing, consisting of a closed chamber where the waterproofing product is sprayed. The chamber consists of a closed metal body inside which a perforated drum is placed, rotating on a horizontal axis driven by an electric motor, with a spray nebulization system installed on the closing door and powered by a dedicated external system.

The machine can be set, creating customized cycles, by means of a special PLC installed on the machine itself.

The basket can contain up to a maximum of 4 kg of dry fabric/garments, but a maximum load of 3 kg is used in the method according to the invention, so that the distribution of the waterproofing product is carried out uniformly on the textile products being processed.

A spray machine useable for the present invention is the model G1 35 HD/HW with Core system from the company Tonello s.r.l.

Preferably, step C) includes the following operating parameters:
- spraying air pressure 2 bar
- waterproofing composition pressure 2.6 bar
- basket rotation start
   20 right/left revolutions
   2 sec pause
   27 rpm drum rotation speed
- first maintenance of basket rotation 0.5 minutes
- waterproofing composition spraying time 15 minutes
- second drum rotation maintenance 5 minutes.

Step E) of drying the waterproofed textile products is carried out by hanging the waterproofed and wet textile product and allowing it to dry in a heated and ventilated place, for example in a forced air circulation oven or, with reference to figure 1, in a heated chamber 6.

The drying has the purpose of "wilting" the waterproofing resin before the cross-linking step, with the purpose of preserving it from the friction imparted by the machine used for the subsequent cross-linking, which otherwise could partially remove it.

Step F) of heat-treating the waterproofed and dried textile products comprises treating said textile products at a temperature between 40°C and 80°C and for a time between 15 and 40 minutes.

The selection of the temperature/time combination will be made based on the different features of the textile products and in particular of the resistance thereof to heat treatment, as reported on the textile product label or tag. For example, the most delicate textile products will undergo a treatment at no more than 45°C for a longer time, for example 35 minutes. Conversely, the most resistant textile products will undergo a treatment at 60°C or even up to 80°C, but for shorter times, for example about 15 minutes.

The heat treatment allows the cross-linking of the aminated dendrimers with the poly-isocyanates, so as to form a protective resin on the treated fabric.

In preferred embodiments, with reference to figure 1, step C) is carried out using a dryer 7 (or tumbler), for example the dryer model Essicat SW 50 from the company Renzacci S.p.A. Such a machine is configured for discontinuous processing, and consists of a closed and heated metal body, in which a perforated metal basket is inserted which rotates on a horizontal axis driven by an electric motor. The internal heating of the machine is obtained by a heat exchanger, inside which steam circulates.

However, such a dryer cannot be used for delicate textile products.

### EXPERIMENTAL PART

Tests were carried out on the same garment (ski suit) with an initial spray test of 0, comparing the treatment according to the method of the invention with the main products (consumers) on the market for domestic use (TX direct spray Nikwax on, TX direct wash Nikwax, Organotex Wash In and Grangers Performance Repel Plus).

Application methods of products for domestic use:
a) Organotex Wash In: 100 ml in a washing cycle in the washing machine at 40°C;
b) Nikwax spray: 2 spraying passages on a wet garment;
c) Nikwax Wash On: 2 caps (about 100 ml) in a washing cycle in the washing machine at 30°C;
d) Grangers Repel plus: spray application from a distance of 15 cm on a wet garment.

Subsequent washing methods (with detergents recommended by the manufacturers for the various waterproofing treatments:
a) Organotex Bio Care detergent: 100 ml in a washing cycle in the washing machine at 30°C;
b) and c): Nikwax Tech Wash detergent: 2 caps (about 100 ml) in a washing cycle in the washing machine at 30°C;
d) Grangers Wash On: 1 cap (about 50 ml) in a washing cycle in the washing machine at 30°C.

A ski suit was instead subjected to the method of the invention for comparison.

For the garment treated according to the invention, successive washes in the washing machine at 30°C with detergent normally available on the market were carried out.

The samples thus obtained were evaluated by spray test, according to the standard ISO 4920:2013, i.e., by spraying 250 ml of distilled or completely deionized water on the sample to be tested which must be fixed on a circle and placed at an angle of 45° so that the center of the sample is 150 mm from the center of the spray nozzle surface. The spray test level is determined by visually comparing the sample with photographic or descriptive standards. The classification according to the spray test can be defined as follows:

| | |
|---|---|
| 0 | Complete wetting of the entire sample surface |
| 50 | Complete wetting of the entire sample surface beyond the spray points |
| 70 | Partial wetting of the sample surface beyond the spray points |
| 80 | Wetting of the sample surface at the spray points |
| 90 | Light and random wetting of the sample surface |
| 100 | No wetting |

The results obtained with the products for domestic use and those obtained according to the invention are reported below:

| **Spray test** | **Method of the inventio n** | **Organotex** | **Nikwax spray** | **Nikwax Wash On** | **Grangers** |
|---|---|---|---|---|---|
| Time 0 | 90-100 | 90 | 70 | 50 | 90-100 |
| After 1 wash | 90-100 | 0 | 0 | 0 | 90-100 |
| After 5 washes | 90 | | | | 70 |
| After 10 washes | 90 | - | - | - | 0 |

The tests carried out not only show a better waterproofing effect at time 0 (i.e., immediately after the application of the method of the invention), but above all a greater persistence of the effect (increased resistance to washing).

Further advantages of the method according to the invention can be found in the fact that the waterproofing step is carried out without the use of water, while for two of the domestic products tested (Organotex and Nikwax Wash On) the waterproofing application is carried out during a washing cycle in the washing machine with consequent water consumption (average water consumption: 40-50 liters per cycle).

The product for domestic use with spray application (Nikwax spray) instead does not require the use of water from the washing cycle in the washing machine, but includes the exposure of the user to the possible vapors deriving from the spray itself. Furthermore, the spray application does not allow to have a precise control of the amount of product used.

The waterproofing according to the method of the invention occurs in a closed environment, without exposure of the worker to possible vapors, and with a precise dosage of the waterproofing composition.

It is apparent that only a few particular embodiments of the present invention have been described, to which those skilled in the art will be able to make all of the necessary changes for the adaptation thereof to particular applications, without however departing from the scope of protection of the present invention.

## Claims

1. A method for giving water-repellent properties to textile products, comprising the following operating steps:
A) providing new or used textile products;
B) washing said textile products;
C) drying said washed textile products;
D) waterproofing said dried textile products;
E) drying said waterproofed textile products;
F) heat-treating the waterproofed and dried textile products, **characterized in that** the waterproofing step D) is carried out, preferably by spraying, using a waterproofing composition comprising or consisting of:
i) a suspension or nanosuspension of silicon dioxide;
ii) hydrocarbon dendrimers or aminated hydrocarbon dendrimers in a hydrocarbon matrix;
iii) polyfunctional isocyanate polymer containing hexamethylene diisocyanate.

2. The method according to claim 1, wherein the washing step B) comprises the following steps:
b1) washing the textile products with a detergent based on an aqueous mixture of fatty acid starches and dispersants
b2) first rinsing
b3) washing with surfactant extraction agent based on a condensation product of aromatic sulfonic acids and formaldehyde comprising sodium naphthalene sulfonate
b4) second rinsing
b5) optionally, third rinsing.

3. The method according to claim 2, wherein
the detergent based on an aqueous mixture of fatty acid starches and dispersants is used in an amount between 1 g and 3 g per liter of water.

4. The method according to claim 2 or 3,
wherein the surfactant extraction agent is used in an amount between 1 g and 3 g per liter of water, preferably at a pH of about 5.

5. The method according to claim 4, wherein step B) includes:
i) weighing the dry textile products
ii) filling the machine with an amount of softened water at a ratio of 40:1 on the weight of the dry textile product
iii) adding a 2 g amount of detergent, preferably Tanaterge EF, for each L of bath
iv) actuating the bath movement blade, so as to circulate and homogenize the washing bath
v) adding the textile products, preferably one at a time so that they are evenly distributed in the tank
vi) heating the bath up to a temperature of 30-40°C, for example based on the maintenance tag of the textile products
vii) once the treatment temperature has been reached, allowing the bath and textile products to circulate for about 20 minutes
viii) after this time, draining the bath, leaving the textile products therein
ix) rinsing the washed textile products by filling the machine with untreated water at a ratio of 40:1 on the weight of the dry textile products, at room temperature and for a residence time of about 10 minutes
x) removing the textile products from the tank
xi) draining the bath
xii) filling the machine with an amount of softened water at a ratio of 40:1 on the weight of the dry textile products
xiii) adding a 2 g amount of surfactant extraction agent, preferably Erional RF, pre-diluted 1:1 with cold softened water, for each L of bath
xiv) controlling the pH value of the bath, for example using a litmus paper
xv) if needed, adjusting the bath to the pH value ~ 5 by adding an appropriate amount of 80% acetic acid
xvi) inserting the wet textile products removed in step 10 into the tank
xvii) increasing the temperature to no more than 40°C
xviii) allowing the textile products turn in the bath at this temperature for about 30 minutes xix) draining the bath
xx) filling the machine with an amount of untreated water at a ratio of 40:1 on the weight of the dry textile products
xxi) cold-treating the textile products for about 10 minutes
xxii) based on the type of textile products being processed, considering whether to repeat another rinse
xxiii) removing the textile products from the tank and placing them on special carriages.

6. The method according to any one of claims 1 to 5, wherein the drying step C) comprises the following steps:
c1) spinning the textile products washed according to step B)
c2) drying the spun textile products.

7. The method according to claim 6, wherein:
- in step c1), the spinning speed is no higher than 500 rpm, and/or
- in step c2), the drying temperature is no higher than 40°C.

8. The method according to claim 1, wherein the waterproofing composition comprises or consists of:
- 75-85% by weight of silicon dioxide suspension or nanosuspension
- 14-23% by weight of hydrocarbon dendrimers or aminated hydrocarbon dendrimers in a hydrocarbon matrix
- 0.5-3% by weight of polyfunctional isocyanate polymer solution containing hexamethylene diisocyanate.

9. The method according to any one of claims 1 to 8, wherein the amount of waterproofing composition used in step C) is 70-90% by weight, or about 80% by weight, with respect to the weight of the dry textile products.

10. The method according to any one of claims 1 to 9, wherein the step F) of heat-treating the waterproofed and dried textile products comprises treating said textile products at a temperature between 40°C and 80°C and for a time between 15 and 40 minutes.

## Patentansprüche

1. Verfahren zum Verleihen von wasserabweisenden Eigenschaften an Textilprodukte, umfassend die folgenden Arbeitsschritte:
A) Bereitstellen von neuen oder gebrauchten Textilprodukten;
B) Waschen der Textilprodukte;
C) Trocknen der gewaschenen Textilprodukte;
D) Wasserabdichten der getrockneten Textilprodukte;
E) Trocknen der wasserabgedichteten Textilprodukte;
F) Wärmebehandlung der wasserabgedichteten und getrockneten Textilprodukte,
**dadurch gekennzeichnet, dass** der Wasserabdichtungsschritt D), vorzugsweise durch Sprühen, unter Verwendung einer Wasserabdichtungs-Zusammensetzung durchgeführt wird, die Folgendes umfasst oder daraus besteht:
i) eine Suspension oder Nanosuspension von Siliziumdioxid;
ii) Kohlenwasserstoff-Dendrimere oder aminierte Kohlenwasserstoff-Dendrimere in einer Kohlenwasserstoffmatrix;
iii) polyfunktionelles Isocyanatpolymer, das Hexamethylendiisocyanat enthält.

2. Verfahren nach Anspruch 1, wobei der Waschschritt B) die folgenden Schritte umfasst:
b1) Waschen der Textilprodukte mit einem Detergens auf der Basis einer wässrigen Mischung aus Fettsäurestärken und Dispergiermitteln
b2) erste Spülung
b3) Waschen mit einem Tensid-Extraktionsmittel auf der Basis eines Kondensationsprodukts von aromatischen Sulfonsäuren und Formaldehyd, das Natriumnaphthalinsulfonat umfasst
b4) zweite Spülung
b5) gegebenenfalls dritte Spülung.

3. Verfahren nach Anspruch 2, wobei das Detergens auf Basis einer wässrigen Mischung aus Fettsäurestärken und Dispergiermitteln in einer Menge zwischen 1 g und 3 g pro Liter Wasser verwendet wird.

4. Verfahren nach Anspruch 2 oder 3, wobei das Tensid-Extraktionsmittel in einer Menge zwischen 1 g und 3 g pro Liter Wasser verwendet wird, vorzugsweise bei einem pH-Wert von etwa 5.

5. Verfahren nach Anspruch 4, wobei Schritt B) beinhaltet:
i) Wiegen der trockenen Textilprodukte
ii) Befüllen der Maschine mit einer Menge an enthärtetem Wasser in einem Verhältnis von 40 : 1 zum Gewicht des trockenen Textilprodukts
iii) Zugeben einer Menge von 2 g Detergens, vorzugsweise Tanaterge EF, für jeden L des Bades
iv) Betätigen des Badbewegungsflügels, um das Waschbad umzuwälzen und zu homogenisieren
v) Zugeben der Textilprodukte, vorzugsweise eines nach dem anderen, so dass sie gleichmäßig im Tank verteilt werden
vi) Heizen des Bades auf eine Temperatur von 30-40°C, z.B. in Abhängigkeit von der Pflegekennzeichnung der Textilprodukte
vii) nach Erreichen der Behandlungstemperatur Umwälzen des Bades und der Textilprodukte für etwa 20 Minuten
viii) nach dieser Zeit Ablassen des Bades, wobei die Textilprodukte darin verbleiben
ix) Spülen der gewaschenen Textilprodukte durch Befüllen der Maschine mit unbehandeltem Wasser in einem Verhältnis von 40 : 1 zum Gewicht der trockenen Textilprodukte, bei Raumtemperatur und für eine Verweildauer von etwa 10 Minuten
x) Entnehmen der Textilprodukte aus dem Tank
xi) Ablassen des Bades
xii) Befüllen der Maschine mit einer Menge enthärteten Wassers in einem Verhältnis von 40 : 1 zum Gewicht der trockenen Textilprodukte
xiii) Zugeben einer Menge von 2 g Tensid-Extraktionsmittel, vorzugsweise Erional RF, das im Verhältnis 1 : 1 mit kaltem, enthärtetem Wasser vorverdünnt ist, für jeden L Bad
xiv) Kontrolle des pH-Wertes des Bades, z.B. mit einem Lackmuspapier
xv) falls erforderlich, Einstellen des Bades auf einen pH-Wert von ~ 5 durch Zugabe einer entsprechenden Menge 80%iger Essigsäure
xvi) Einbringen der in Schritt 10 entnommenen nassen Textilprodukte in den Tank
xvii) Erhöhen der Temperatur auf nicht mehr als 40°C
xviii) Wenden der Textilprodukte im Bad bei dieser Temperatur für etwa 30 Minuten
xix) Ablassen des Bades
xx) Befüllen der Maschine mit einer Menge an unbehandelten Wassers in einem Verhältnis von 40 : 1 zum Gewicht der trockenen Textilprodukte
xxi) Kaltbehandlung der Textilprodukte für etwa 10 Minuten
xxii) je nach Art der verarbeiteten Textilprodukte Prüfen, ob eine weitere Spülung erforderlich ist
xxiii) Entnehmen der Textilprodukte aus dem Tank und Platzierung auf speziellen Wagen.

6. Verfahren nach einem der Ansprüche 1 bis 5, wobei der Trocknungsschritt C) die folgenden Schritte umfasst:
c1) Spinnen der gemäß Schritt B) gewaschenen Textilprodukte
c2) Trocknen der gesponnenen Textilprodukte.

7. Verfahren nach Anspruch 6, wobei:
- in Schritt c1) die Spinngeschwindigkeit nicht höher als 500 U/min ist, und/oder
- in Schritt c2) die Trocknungstemperatur nicht höher als 40°C ist.

8. Verfahren nach Anspruch 1, wobei die wasserabdichtende Zusammensetzung umfasst oder besteht aus:
- 75-85 Gew.-% Siliciumdioxid-Suspension oder -Nanosuspension
- 14-23 Gew.-% Kohlenwasserstoff-Dendrimere oder aminierte Kohlenwasserstoff-Dendrimere in einer Kohlenwasserstoffmatrix
- 0,5-3 Gew.-% einer polyfunktionellen Isocyanat-Polymerlösung, die Hexamethylendiisocyanat enthält.

9. Verfahren nach einem der Ansprüche 1 bis 8, wobei die Menge der in Schritt C) verwendeten wasserabdichtenden Zusammensetzung 70-90 Gew.-% oder etwa 80 Gew.-% beträgt, bezogen auf das Gewicht der trockenen Textilprodukte.

10. Verfahren nach einem der Ansprüche 1 bis 9, wobei der Schritt F) der Wärmebehandlung der wasserabgedichteten und getrockneten Textilprodukte die Behandlung der Textilprodukte bei einer Temperatur zwischen 40°C und 80°C und für eine Zeit zwischen 15 und 40 Minuten umfasst.

## Revendications

1. Procédé pour donner des propriétés hydrofuges à des produits textiles, comprenant les étapes de fonctionnement suivantes :
A) la fourniture de produits textiles neufs ou usagés ;
B) le lavage desdits produits textiles ;
C) le séchage desdits produits textiles lavés ;
D) l'imperméabilisation desdits produits textiles séchés ;
E) le séchage desdits produits textiles imperméabilisés ;
F) le traitement thermique des produits textiles imperméabilisés et séchés, **caractérisé en ce que** l'étape d'imperméabilisation D) est réalisée, de préférence par pulvérisation, au moyen d'une composition d'imperméabilisation comprenant ou constituée de :
i) une suspension ou nanosuspension de dioxyde de silicium ;
ii) des dendrimères d'hydrocarbure ou dendrimères d'hydrocarbure aminé dans une matrice d'hydrocarbure ;
iii) un polymère isocyanate polyfonctionnel contenant du diisocyanate d'hexaméthylène.

2. Procédé selon la revendication 1, dans lequel l'étape de lavage B) comprend les étapes suivantes :
b1) le lavage des produits textiles avec un détergent à base d'un mélange aqueux d'amidons d'acide gras et de dispersants
b2) un premier rinçage
b3) le lavage avec un agent d'extraction de tensio-actif à base d'un produit de condensation d'acides sulfoniques aromatiques et de formaldéhyde comprenant du sulfonate de naphthalène de sodium
b4) un deuxième rinçage
b5) éventuellement, un troisième rinçage.

3. Procédé selon la revendication 2, dans lequel le détergent à base d'un mélange aqueux d'amidons d'acide gras et de dispersants est utilisé dans une quantité comprise entre 1 g et 3 g par litre d'eau.

4. Procédé selon la revendication 2 ou 3, dans lequel l'agent d'extraction de tensio-actif est utilisé dans une quantité comprise entre 1 g et 3 g par litre d'eau, de préférence à un pH d'environ 5.

5. Procédé selon la revendication 4, dans lequel l'étape B) comporte :
i) le pesage des produits textiles secs
ii) le remplissage de la machine avec une quantité d'eau adoucie à un rapport de 40:1 sur le poids du produit textile sec
iii) l'ajout d'une quantité de 2 g de détergent, de préférence de Tanaterge EF, pour chaque L de bain
iv) l'actionnement de la pale de mouvement de bain, de manière à faire circuler et homogénéiser le bain de lavage
v) l'ajout des produits textiles, de préférence un par un de sorte qu'ils sont répartis uniformément dans le réservoir
vi) le chauffage du bain jusqu'à une température de 30-40 °C, par exemple sur la base de l'étiquette d'entretien des produits textiles
vii) une fois que la température de traitement a été atteinte, le fait de faire circuler le bain et les produits textiles pendant environ 20 minutes
viii) après ce temps, la vidange du bain, en laissant les produits textiles dans celui-ci
ix) le rinçage des produits textiles lavés par remplissage de la machine avec de l'eau non traitée à un rapport de 40:1 sur le poids des produits textiles secs, à température ambiante et pendant un temps de séjour d'environ 10 minutes
x) le retrait des produits textiles du réservoir
xi) la vidange du bain
xii) le remplissage de la machine avec une quantité d'eau adoucie à un rapport de 40:1 sur le poids des produits textiles secs
xiii) l'ajout d'une quantité de 2 g d'agent d'extraction de tensio-actif, de préférence d'Erional RF, prédilué à 1:1 avec de l'eau adoucie froide, pour chaque L de bain
xiv) la régulation de la valeur de pH du bain, par exemple au moyen d'un papier de tournesol
xv) si nécessaire, l'ajustement du bain à la valeur de pH ~ 5 par ajout d'une quantité appropriée de 80 % d'acide acétique
xvi) l'insertion des produits textiles humides retirés dans l'étape 10 dans le réservoir
xvii) l'augmentation de la température à pas plus de 40 °C
xviii) le fait de faire tourner les produits textiles dans le bain à cette température pendant environ 30 minutes
xix) la vidange du bain
xx) le remplissage de la machine avec une quantité d'eau non traitée à un rapport de 40:1 sur le poids des produits textiles secs
xxi) le traitement à froid des produits textiles pendant environ 10 minutes
xxii) sur la base du type de produits textiles en train d'être traités, le fait d'estimer s'il est nécessaire de répéter un autre rinçage
xxiii) le retrait des produits textiles du réservoir et leur placement sur des chariots spéciaux.

6. Procédé selon l'une quelconque des revendications 1 à 5, dans lequel l'étape de séchage C) comprend les étapes suivantes :
c1) l'essorage des produits textiles lavés conformément à l'étape B)
c2) le séchage des produits textiles essorés.

7. Procédé selon la revendication 6, dans lequel :
- dans l'étape c1), la vitesse d'essorage n'est pas supérieure à 500 tr/min, et/ou
- dans l'étape c2), la température de séchage n'est pas supérieure à 40 °C.

8. Procédé selon la revendication 1, dans lequel la composition d'imperméabilisation comprend ou est constituée de :
- 75-85 % en poids d'une suspension ou nanosuspension de dioxyde de silicium
- 14-23 % en poids de dendrimères d'hydrocarbure ou de dendrimères d'hydrocarbure aminé dans une matrice d'hydrocarbure
- 0,5-3 % en poids d'une solution de polymère isocyanate polyfonctionnel contenant du diisocyanate d'hexaméthylène.

9. Procédé selon l'une quelconque des revendications 1 à 8,
dans lequel la quantité de composition d'imperméabilisation utilisée dans l'étape C) est 70-90 % en poids, ou environ 80 % en poids, par rapport au poids des produits textiles secs.

10. Procédé selon l'une quelconque des revendications 1 à 9, dans lequel l'étape F) de traitement thermique des produits textiles imperméabilisés et séchés comprend le traitement desdits produits textiles à une température comprise entre 40 °C et 80 °C et pendant un temps compris entre 15 et 40 minutes.
